

# UNITED STATES PATENT OFFICE.

JOHN F. LOVEJOY, OF NEW YORK, N. Y., ASSIGNOR OF ONE-HALF TO ABE STEIN,  
OF NEW YORK, N. Y.

## METHOD OF PRODUCING ANTHRACITE BRIQUETS.

No. 921,550.

Specification of Letters Patent.

Patented May 11, 1909.

Application filed March 5, 1906. Serial No. 304,342.

*To all whom it may concern:*

Be it known that I, JOHN F. LOVEJOY, a citizen of the United States, and a resident of the city of New York, county of New York, and State of New York, have invented a new and useful Improvement in Methods of Producing Anthracite Briquets, of which the following is a specification.

The aim of my invention is to utilize anthracite coal dust or culm in the production of freely combustible briquets adapted to retain their form during combustion and to gradually burn away on the exterior.

It is well known to those familiar with the subject that anthracite culm has been accumulating at the American mines for many years, and that it now exists in vast quantities as a useless material which is disposed of by the mining companies at great expense by piling it in huge banks at great height or by distributing it in the abandoned mines.

Many attempts have been made by official commissions of the State of Pennsylvania and others to produce briquets from this material, but without success. Briquets of anthracite coal alone are not and never have been known to commerce.

As heretofore produced, the briquets would either suddenly disintegrate on being subjected to the heat of the fire or, on the other hand, they would melt down or assume a pasty condition. In either case the maintenance of an open fire-bed through which air could pass to maintain combustion was impossible, and consequently the briquets were useless.

In carrying my invention into effect I provide coal tar pitch of a high melting point, preferably 150 to 160 degrees Fahrenheit, and by means of suitable apparatus maintain the same in fluid condition, ready for use.

The culm or coal dust to be used is passed through a heating or retorting apparatus of any suitable character, preferably through a long inclined rotating cylinder, and subjected during its passage to a heat sufficient to drive off all moisture and raise the temperature of the coal to a degree materially above that at which the pitch melts. This is best effected by delivering the flame and hot gases of combustion from a suitable coal or other fire through the cylinder while the coal is also passing slowly therethrough.

The temperature to which the coal is

subjected may be modified to some extent, but with most Pennsylvania anthracites I find a temperature of from 250 to 350 degrees Fahrenheit gives the best results, 300 to 310 degrees being the temperature I generally employ. After the coal has been treated as above and while it is still in a highly heated condition, at a temperature preferably near 280 degrees Fahrenheit, I add from 8 to 10 per cent. of the molten pitch at about 240 degrees Fahrenheit, thoroughly agitating the mass until it is of a homogeneous character and until the particles of coal are coated with a thin film of pitch. The mass is cooled or permitted to cool until it is cohesive and of suitable consistency to admit of its being molded into the required forms. While still in a heated condition, preferably from 160 to 220 degrees Fahrenheit, it is delivered to a molding or briquetting machine of any suitable character, adapted to apply severe pressure, and is formed thereby into briquets or bodies of any suitable size and form. The resulting briquets on being cooled or permitted to cool acquire extreme hardness and tenacity and may be handled freely and violently without danger of disintegration.

When briquets produced as above are placed in the fire they will readily ignite and will burn away gradually on the exterior while retaining their form and solidity, thus permitting the maintenance of an open or pervious bed through which a free draft may be maintained to keep up combustion.

In the formation of the briquets it is found that the application of a very severe pressure has the effect of giving to the briquets greater hardness and greater powers of resistance against fracture than when they are molded under moderate pressure.

Having described my invention, what I claim is:

1. The method of producing briquets from anthracite coal consisting in heating the coal to a temperature of from 250 to 350 degrees Fahrenheit, combining therewith molten pitch at about 240 degrees Fahrenheit, thoroughly agitating the mass, and finally forming the same, under severe pressure, at a temperature of from 160 to 220 degrees Fahrenheit, into briquets.

2. The method of producing combustible briquets from anthracite coal consisting in subjecting the coal to a temperature of from

250 to 350 degrees Fahrenheit, thereafter combining with the coal while at a temperature of about 280 degrees Fahrenheit, molten pitch having a melting point of about 160 degrees Fahrenheit and a temperature of about 240 degrees Fahrenheit, subjecting the mass to thorough agitation and thereafter molding the same, at a temperature of about 160 degrees Fahrenheit to 220 degrees Fahrenheit, into briquets.

3. The method of producing anthracite briquets consisting in combining highly heated coal in the absence of moisture with

molten refractory pitch at a high temperature, and agitating the mass until it is of a homogeneous character, and causing or permitting the mass to partially cool, and finally molding the mass into briquets under severe pressure.

In testimony whereof I hereunto set my hand this 26th day of February, 1906, in the presence of two attesting witnesses.

JOHN F. LOVEJOY.

Witnesses:

P. T. DODGE.

E. J. LAMB.